

## UNITED STATES PATENT OFFICE

2,173,218

METHOD FOR WHETTING FILES, RASPS,  
AND THE LIKE

Emanuele Zoppi, Genova, Italy

No Drawing. Application October 18, 1937, Serial No. 169,753. In Germany November 26, 1936

4 Claims. (Cl. 76—24)

This invention relates to a method for whetting files, rasps and the like by etching by means of acid.

It has already been previously proposed to dip 5 files to be whetted into an acid bath without preliminary treatment. This method has the disadvantage that the files were considerably reduced in weight, whilst the whetting obtained only lasted for a very short time. This method 10 is therefore not of practical value.

According to the present invention the grease is first removed from files by treating them in an alkaline bath, they are then treated in a bath of hydrochloric acid, then in a bath of nitric acid, 15 and subsequently in a bath of hydrochloric acid, whereupon any acid which may be adhering thereto is neutralised.

The advantage of the new method resides in the fact that the baths which are used can be 20 produced at low costs, that the files do not lose in weight as a result of the treatment, and the method can be carried out by an unskilled workman. By means of the new method it is possible to obtain in an economical manner sharp 25 and resistant teeth. The method may be carried out for example as follows.

For the removal of grease there is used a soda lye containing 50 g. caustic soda (NaOH) to one litre of water. In this lye the files are boiled for 30 about half an hour. The files are then removed from the lye and rinsed in water and brushed.

The files are then placed into a second bath consisting of 50 parts by weight commercial hydrochloric acid and 50 parts by weight of 35 water. The files are allowed to remain in this bath for 12 hours without the application of heat.

In this bath all adhering substances are removed and the surface is prepared for the succeeding third bath in which the files after having 40 been again rinsed and brushed are placed.

This third bath may be regarded as the renewing bath, it consists of 20 parts by weight of nitric acid of 42° Bé. and 80 parts by weight of water. The files are allowed to remain in this 45 bath for from 5-10 minutes without the application of heat.

During the first moments there are formed fine bubbles which adhere to the points of the teeth, enclose these and protect them against the action 50 of the acid. After 2-3 minutes the bubbles disappear and the bath can attack the whole file. It is important during the treatment in the third bath to repeatedly withdraw the files therefrom and to again immerse them therein.

55 After treatment in the third bath the files are

again washed and brushed. They are then placed for a period of 5-10 minutes into a fourth bath which has the same composition as the second bath. After rinsing and brushing the files are treated in a fifth bath which consists of water 5 and unslaked lime.

For this purpose there are used 5 litre of water and about 100 g. unslaked lime (CaO). It is sufficient if the files are allowed to remain in this bath for about 10-20 minutes. They may however be allowed to remain therein for a longer time (hours or days).

After treatment the files are again washed and brushed. They are then dried for example in saw-dust or by means of an air current and finally 15 greased, preferably with mineral oil.

The washing of the files between the treatments in the separate baths is preferably effected in hot water. Further it is preferable when taking the files from one bath to immediately place them 20 into the washing water and from the washing water immediately into the next bath so that on the passage from one bath to the other they are not exposed to the air for too long a period of time.

25 The files are preferably placed into the baths in a vertical position.

I claim:

1. The method of sharpening files, rasps and the like, which comprises the following steps in 30 the order mentioned, viz: first, subjecting the articles to the de-greasing action of a boiling alkaline bath consisting of 50 g. of NaOH to one litre of water; second, removing the articles from the alkaline bath and rinsing them in water; 35 third, placing the rinsed articles in a bath consisting of approximately equal parts by weight of hydrochloric acid and water, for about twelve hours, at normal temperature; fourth, removing the articles from the hydrochloric acid bath and again rinsing them in water; fifth, placing the rinsed articles in a bath consisting of twenty parts by weight of nitric acid of 42° Bé. and eighty parts by weight of water, for from five to ten 40 minutes, at normal temperature; sixth, removing the articles from the nitric acid bath and after rinsing the same, neutralizing any adhering acid in a milk of lime bath.

2. The method of sharpening files, rasps and the like, which comprises the following steps in 50 the order mentioned, viz: first, subjecting the articles to the de-greasing action of a boiling alkaline bath consisting of 50 g. of NaOH to one litre of water; second, removing the articles from the alkaline bath and rinsing them in water; 55

third, placing the rinsed articles in a bath consisting of approximately equal parts by weight of hydrochloric acid and water, for about twelve hours, at normal temperature; fourth, removing the articles from the hydrochloric acid bath and again rinsing them in water; fifth, placing the rinsed articles in a bath consisting of twenty parts by weight of nitric acid of 42° Bé. and eighty parts by weight of water, for from five to ten minutes, at normal temperature; sixth, removing the articles from the nitric acid bath and after rinsing the same, placing the articles again in a hydrochloric acid bath like that of the third step above; seventh, removing the articles from the last acid bath and after rinsing the articles, neutralizing any acid adhering thereto in a bath of milk of lime.

3. The method of sharpening files, rasps and the like, which comprises the following steps in the order mentioned, viz: first, subjecting the articles to the de-greasing action of a boiling alkaline bath consisting of 50 g. of NaOH to one litre of water; second, removing the articles from the alkaline bath and rinsing them in water; third, placing the rinsed articles in a bath consisting of approximately equal parts by weight of hydrochloric acid and water, for about twelve hours, at normal temperature; fourth, removing the articles from the hydrochloric acid bath and again rinsing them in water; fifth, placing the rinsed articles in a bath consisting of twenty parts by weight of nitric acid of 42° Bé. and eighty parts by weight of water, for from five to

ten minutes, at normal temperature; sixth, removing the articles from the nitric acid bath and after rinsing the same, neutralizing any adhering acid in a milk of lime bath; seventh, removing the articles from the neutralizing bath and washing them and drying them.

4. The method of sharpening files, rasps and the like, which comprises the following steps in the order mentioned, viz: first, subjecting the articles to the de-greasing action of a boiling alkaline bath consisting of 50 g. of NaOH to one litre of water; second, removing the articles from the alkaline bath and rinsing them in water; third, placing the rinsed articles in a bath consisting of approximately equal parts by weight of hydrochloric acid and water, for about twelve hours, at normal temperature; fourth, removing the articles from the hydrochloric acid bath and again rinsing them in water; fifth, placing the rinsed articles in a bath consisting of twenty parts by weight of nitric acid of 42° Bé. and eighty parts by weight of water, for from five to ten minutes, at normal temperature; sixth, removing the articles from the nitric acid bath and after rinsing the same, placing the articles again in a hydrochloric acid bath like that of the third step above; seventh, removing the articles from the last acid bath and after rinsing the articles, neutralizing any acid adhering thereto in a bath of milk of lime; eighth, removing the articles from the neutralizing bath and washing them and drying them.

ZOPPI, EMANUELE.